

## UNITED STATES PATENT OFFICE

2,200,383

TEXTILE MATERIAL AND METHOD OF  
MAKING SAMECyril M. Croft, Cumberland, Md., assignor to  
Celanese Corporation of America, a corpora-  
tion of DelawareNo Drawing. Application April 6, 1938,  
Serial No. 200,433

6 Claims. (Cl. 8—130)

This invention relates to the treatment of fabrics, yarns, filaments and like textile materials containing an organic ester of cellulose with a saponifying agent to obtain fabrics, yarns and filaments having an affinity for acid and basic dyestuffs employed in dyeing and printing cotton fabrics which dyestuffs have little or no affinity for organic derivative of cellulose material.

10 An object of the invention is the saponification of fabrics, particularly those formed from yarns containing an organic ester of cellulose, which yarns have a high degree of twist or offer resistance to the penetration of fluid treating mediums 15 for other reasons. Other objects of this invention will appear from the following detailed description.

It is known that fabrics formed from organic esters of cellulose yarns may be saponified by 20 treatment with a base or a basic salt and that such saponified fabrics develop an affinity for cotton dyestuffs depending upon the extent of saponification and upon the type of saponification treatment. For the purpose of producing cellulose acetate fabrics to be dyed or printed with cotton dyestuffs (direct dyeing acid or vat dyestuffs), it is customary to saponify a cellulose acetate fabric until there is a weight loss of from 10 to 15% although lesser and greater weight 25 losses are regularly effected, say from 5 to 20% or more. In methods employed prior to my invention, only certain types of fabric, i. e. those which are readily penetrated by the saponification fluid, could be saponified, especially on a 30 winch. Other types of fabrics, when dyed, were blotchy or streaked due to uneven saponification or non-uniform type of saponification. For instance, great difficulty was experienced in uniformly saponifying crepe fabrics formed of high- 35 ly twisted (about 65 turns per inch) yarn and closely woven taffetas and satins. I have found that crepe fabrics and other fabrics normally difficult to penetrate with saponifying baths may be uniformly saponified by adding pine oil to the 40 saponifying bath.

Another advantage of this invention is that any 45 type of saponification may be produced. The speed of saponification, among other things, controls the type of saponification, i. e. whether the saponification is limited to the surface of the 50 filaments or fibers that make up the yarn, or whether the saponification is through and through saponification. Prior to this invention it was necessary to treat crepe fabrics, taffetas and satin fabrics with a slow saponifying bath

for long periods of time to obtain uniform saponification. This resulted in a low dye affinity change per weight loss. Long saponification treatments not only produce a through and through type of saponification, which is not always desired, but also are likely to be injurious to the fabric, especially when treating crepe fabrics prior to their treatment in creping baths. However, I have found that with the use of pine oil in the bath it is not necessary to saponify 10 slowly by cooling the bath and/or diluting the concentration of effective saponifying agents to obtain a uniform saponification. By employing this invention, uniform saponification may be obtained employing more concentrated effective 15 saponifying agents, thus greatly reducing the time of treatment of the fabric in the bath.

In accordance with my invention, I saponify fabrics or other textile materials made of or containing an organic ester of cellulose by treating the same with a bath containing pine oil and a saponifying agent such as alkali, or ammonia hydroxides or carbonates, or organic ammonium or amine compounds having saponifying properties, or inorganic or organic salts having a 20 saponifying action. Examples of suitable saponifying agents are sodium, potassium or ammonia hydroxide, carbonate or acetate; di- or tri-ethanolamine; secondary and tertiary alkyl substituted ammonium compounds, etc. The degree of saponification may be from less than 3% by weight loss to substantially complete saponification. However, the invention is particularly applicable to saponification which effects a weight loss of from 5 to 20%, based upon the weight of 25 the organic ester of cellulose in the fabric, and to a quick saponification which greatly modifies the surface of the filaments and leaves the center of the filaments substantially unchanged. This produces a fabric having an affinity for cotton 30 dyestuffs yet one which retains to a great extent the thermoplastic properties of the derivative of cellulose and which retains the original properties of the fabric with respect to beauty of drape, 35 luster, hand, etc.

This invention is applicable to textile materials such as fabrics, yarns, etc., that are made of or contain organic esters of cellulose. Examples of organic esters of cellulose are cellulose acetate, cellulose formate, cellulose propionate and cellulose butyrate. Fabrics may be made entirely of yarns containing organic esters of cellulose or they may be formed from such yarns together with yarns of other materials such as reconstituted or regenerated cellulose, cotton, wool, 40 45 50

silk, etc. The invention is of especial importance in the saponification of crepe fabrics which may contain, besides the organic ester of cellulose threads, threads of regenerated or reconstituted cellulose. These may alternate in any desired manner to produce the crepe effect desired.

A fabric formed of substantially all organic ester of cellulose yarns may be saponified by employing a winch, the treating bath of which may comprise from 1 to 20 or more times the weight of the fabric of water containing from 5 to 20% or more, based on the weight of the fabric, of a saponifying agent equivalent in strength to that of sodium hydroxide. This aqueous bath also contains from 0.5 to 2 grams per liter of pine oil. The time and temperature of the bath may be so regulated to give the desired degree and type of saponification. The pine oil in the bath prevents the fabric from floating and also effects a rapid penetration of the saponifying agent into the interstices of the fabric. Although one or more grams per liter of soap may be employed, it is preferable to use only the pine oil as the penetrating agent as soap tends to froth and prevent the fabric from sinking. The floating of the fabric, due to the froth formed when employing soap, tends to create a blotchy pattern and warp streaks where the saponifying agent has not had a chance to act upon the fabric for the same length of time as that part of the fabric which is not caused to float.

As an illustration of my invention, but without being limited thereto, the following example is given:

**35 Example**

100 pounds of fabric made by weaving yarns of cellulose acetate twisted to 65 turns per inch is treated on the winch with a bath containing 25 gallons of water, 12 pounds of sodium carbonate and 1 gram per liter of pine oil. The fabric is treated at room temperature for two hours, ef-

fecting a weight loss to the fabric of between 10 and 15%. The fabric is dyed with a cotton dyeing dyestuff and the fabric thus dyed is of uniform color, free of blotchiness and warp streaks produced by uneven dye affinity.

It is to be understood that the foregoing detailed description is merely given by way of illustration and that many variations may be made therein without departing from the spirit of my invention.

Having described my invention, what I desire to secure by Letters Patent is:

1. In a process of saponifying textile materials containing an organic ester of cellulose, the steps of subjecting the fabric to a saponifying bath 15 consisting of a saponifying agent and pine oil.

2. In a process of saponifying textile materials containing cellulose acetate, the steps of subjecting the fabric to a saponifying bath consisting of a saponifying agent and pine oil.

3. In a process of saponifying textile materials containing an organic ester of cellulose, the steps of subjecting the fabric to a saponifying bath 25 consisting of a saponifying agent and 0.5 to 2 grams per liter of pine oil.

4. In a process of saponifying textile materials containing cellulose acetate, the steps of subjecting the fabric to a saponifying bath consisting of a saponifying agent and 0.5 to 2 grams per liter of pine oil.

5. In a process of saponifying textile materials containing cellulose acetate, the steps of subjecting the fabric to a saponifying bath consisting of sodium carbonate and pine oil.

6. In a process of saponifying textile materials containing cellulose acetate, the steps of subjecting the fabric to a saponifying bath consisting of sodium carbonate and 0.5 to 2 grams per liter of pine oil.

CYRIL M. CROFT. 40

10

20

25

30

40